

May 18, 1965

L. L. BURNS, JR

3,184,329

INSULATION

Filed Dec. 16, 1960



Fig. 1.



Fig. 2.



Fig. 3.



Fig. 4.

INVENTOR.  
LESLIE L. BURNS, JR.  
BY *John V. Regan*  
ATTORNEY

3,184,329

## INSULATION

Leslie L. Burns, Jr., Princeton, N.J., assignor to Radio Corporation of America, a corporation of Delaware  
Filed Dec. 16, 1960, Ser. No. 76,288  
7 Claims. (Cl. 117—106)

This application deals with the problem of providing very thin, evaporated layers (films) of insulating material which are free of pin holes. While not restricted thereto, the solution to this problem is of considerable importance in the making of certain superconductor electrical circuits, and in other applications, such as the making of capacitors, for example.

There are a number of electrical circuit applications in which thin insulator films are useful. For example, in superconductor circuits it may be desired to provide very close coupling between a superconducting lead carrying a drive current and an element such as a sheet of superconductor material, a portion of which it is desired to drive from its superconducting to its normal state. A thin insulator film makes the close spacing possible. Capacitor technology is another area in which close spacing between metal layers may be desired—here for the purpose of increasing capacitance. Thin insulating films make the close spacing possible.

Vacuum evaporation is one method for obtaining thin films. In this method, the surface on which it is desired to deposit the film is placed in a vacuum chamber. The insulator material to be deposited is placed in a basket or crucible, also in the vacuum chamber and is heated to a high temperature. The evaporated insulator material then deposits on the surface in the form of a film.

Unfortunately, vacuum evaporation has not proved to be an entirely satisfactory method of producing thin films. Films produced in this manner have very minute holes therein which hereafter are termed, "pin holes." Since the film normally occupies the space between two layers of metal, one on which the film is deposited and the other deposited on the other surface of the film, the pin holes provide a path through which the deposited metal extends. The metal extending into the pin holes produces a short circuit between metal layers thereby greatly lessening or destroying the insulating property of the film.

There have been a number of theories to explain the pin holes and solutions based on these theories have been attempted. Perhaps the most accepted theory up to the present has been that very small particles are present on the surface on which the insulator layer is formed. These particles were thought to produce a shadow area which remained free of insulation when the evaporated insulator was deposited on the surface. This shadow area was thought to be the pin hole. Based on this theory, a number of solutions, none of which were successful, were attempted to overcome the problem. For example, in one method insulating material was vacuum evaporated simultaneously from two spaced baskets in an attempt to make the insulating material particles land on the surface at different angles and cover the shadow area. In another method, the basket containing the insulating material was moved to various locations in the vacuum chamber during the vacuum evaporation.

It is believed that the theory above and others which have been advanced are incorrect. Two new theories, either one of which can explain the presence of pin holes, are discussed in greater detail below. However, whether or not either one of these theories is correct, they have provided a clue toward the solution of this problem and,

in any case, it has been found that the method of producing films disclosed herein does solve the problem.

According to the present invention, a film of insulating material is applied in two separate steps. First, a thin layer of the material is evaporated onto the surface it is desired to cover. This evaporation takes place in a vacuum. The pressure is then raised. The pressure is then lowered to that of a vacuum again and a second layer of insulating material is applied over the first. It is found that the film produced in this manner is free of pin holes over a very large area.

The invention is described in greater detail below and is illustrated in the following drawing of which:

FIG. 1 is a cross-sectional view of the way in which a thin insulator film on a metal surface is believed to appear during the vacuum evaporation of the insulator film;

FIG. 2 is a cross-sectional view of the film of FIG. 1 at atmospheric pressure;

FIG. 3 is a cross-sectional view of an insulator film according to the present invention; and

FIG. 4 is a cross-sectional view of two vacuum deposited metal films with an insulator film according to the present invention between.

FIG. 1 shows a metal film 10 on which is deposited an insulator film 11. The film is deposited in conventional manner, that is by vacuum evaporating the insulator material in the manner briefly discussed in the introductory portion of the specification. For superconductor applications, silicon monoxide (SiO) has been found to be especially suitable. The vacuum evaporation is preferably carried out at a rather low pressure such as  $10^{-5}$  or  $10^{-6}$  millimeters of mercury. However, any pressure lower than  $10^{-4}$  millimeters of mercury is satisfactory. The silicon monoxide is located in a crucible within the vacuum chamber and is heated to a temperature of 1290 degrees C. The vacuum evaporation is continued until a desired thickness such as 1,500 Angstroms is reached. The thickness can be determined by timing the heating step or alternatively by allowing the silicon monoxide to simultaneously deposit on the desired substrate and a quartz crystal that is in an electrical oscillating circuit. As the silicon monoxide is deposited on the crystal, the frequency of oscillation is changed. By measuring the frequency change, the evaporation can be terminated when the desired thickness is reached.

It is believed that during the vacuum evaporation described above, very small bubbles of gas at reduced pressure become included in the film. Two such inclusions are shown at 12 and 13 in FIG. 1. These inclusions occur in a random pattern. It is also believed that when the ambient pressure is increased to atmospheric pressure, these small inclusions implode as is shown at 12 and 13 in FIG. 2. The implosions cause the pin holes which provide passages for subsequent layers of vacuum evaporated metal. Such a layer (not shown) would extend into the pin holes and short circuit with the metal layer 10.

The above theory explains why the previous methods proposed for solving the problem have been unsuccessful. It also explains why increasing the thickness of the layer is not entirely successful either. As a matter of fact, silicon monoxide layers of greater than 20,000 Angstroms have been evaporated in a single step without overcoming the problem of pin holes. Even with layers this thick, it is believed that implosions which still occur cause the undesired pin holes shown in FIG. 2.

According to the present invention, an insulating layer such as silicon monoxide is first formed by vacuum evaporation in the manner already described at a thickness one-half that of the desired thickness. For example, if it is desired to produce a layer 3,000 Angstroms thick, the

first step is to lay down a layer 1,500 Angstroms thick. Then the ambient pressure is increased, preferably to atmospheric pressure. This can be done by permitting air to enter the vacuum chamber. However, this introduces undesired impurities such as moisture. It is preferred that the ambient pressure be raised by admitting a dry inert gas such as dry nitrogen or dry helium. The effect of raising the pressure is to produce the pin holes as shown in FIG. 2. The final step is to reduce the ambient pressure to vacuum again. As already mentioned, the vacuum during the first step and during this step should be lower than  $10^{-4}$  millimeters of mercury. Then a second layer of the insulator material, that is, silicon monoxide is vacuum evaporated onto the first. The second layer also has the gas at low pressure as inclusions therein. However, these occur in a random pattern and this random pattern is different than the random pattern of the pin holes in the first layer. Thus, when the ambient pressure is raised again, implosions in the second layer produce pin holes in the second layer which do not coincide with the pin holes in the first layer and no continuous path exists between the upper surface of the second insulator layer and the lower surface of the first insulator layer.

FIG. 3 shows an insulator film formed according to the present invention. The metal layer is shown at 14, the first insulator is shown at 15, and the second insulator layer is shown at 16. The first layer has pin holes 17 and 18 therein and the second layer 16 has pin holes 19, 20 and 21 therein. The pin holes in the two layers are not aligned and no path exists from upper surface 22 to lower surface 23. If the two layers are deposited without raising the ambient pressure during the interval between the deposition steps, the improved film does not result. Instead, there are pin holes which extend between opposite surfaces, just as in FIG. 2.

FIG. 4 illustrates a capacitor construction according to the present invention. Layers 25 and 26 are metal and may be tantalum or copper, for example, or some other metal, and layers 27 and 28 together comprise the insulating film formed according to the present invention. The pin holes in each of layers 27 and 28 are not shown. In a practical capacitor, the combined thickness of layers 27 and 28 may be of the order of 500 Angstroms to 1,000 Angstroms. Prior to this invention, it was not possible, so far as Applicant is aware, to obtain large area vacuum deposited insulator films for capacitors of smaller thickness than 20,000 Angstroms.

Silicon monoxide has been given as an example of insulating material which is useful in practicing the present invention. It is, of course, to be understood that the invention is not limited to this specific material. Silicon monoxide is especially suitable for superconducting applications as it does not craze at the low temperatures (several degrees Kelvin) involved. It is also commonly used for capacitor applications. The process of making the film is exactly the same as described above. Other materials which are suitable in practicing the invention are calcium fluoride, silicon dioxide, aluminum oxide, beryllium oxide and magnesium fluoride.

In the discussion above, the two films which are laid down are both of the same material. It is also possible to use different materials for the different layers as, for example, calcium fluoride for one layer and silicon monoxide for the other. It is also sometimes desirable to use more than two insulating films laid down in the manner described. Three or more films may be used, for example, when the total thickness of insulation desired is very small. When the individual layers are very, very thin, many more pin holes are formed and the probability of coincidence between pin holes in the different layers is greater.

While it is believed that the theory advanced above for the occurrence of pin holes in insulator deposits is correct, another theory has been advanced which can possibly explain the pin holes. According to this theory,

randomly occurring electrostatic charges build up on the insulator material being vacuum deposited. Charges also occur in the particles of the material being deposited. If the static charges built up in the insulator layer are the same as those of the insulator particles being deposited, these particles are repelled from the randomly spaced static charge centers and the result is the pin holes already described. According to this theory, when the ambient pressure is raised to atmospheric pressure, the electrostatic charges are dissipated. Accordingly, the second layer which is subsequently vacuum evaporated onto the first is not repelled from the pin hole areas but is instead repelled from different randomly spaced static charge centers.

It is to be understood that the present invention does not depend on either theory discussed above. Both are simply a means to explain why the present invention has given the improved performance it does. The fact is that regardless of the theories, the present invention does operate and does operate successfully. Several hundred films according to the invention have already been fabricated up to the present time and no insulation failures have yet been detected.

What is claimed is:

1. A method of producing a film of insulating material on a surface comprising the steps of evaporating a first layer of an insulating material onto the surface, in vacuum; raising the ambient pressure on the evaporated layer by admitting an inert gas; reducing the ambient pressure on the evaporated layer to that of a vacuum; and evaporating a second layer of the insulating material onto the first.

2. A method as set forth in claim 1, in which said second layer is formed of the same material as said first layer.

3. A method of producing a film of insulating material on a surface comprising the steps of evaporating a first layer of an insulating material onto the surface, in vacuum; raising the ambient pressure on the evaporated layer to atmospheric pressure by admitting an inert gas; reducing the ambient pressure on the evaporated layer to that of a vacuum; and evaporating a second layer of the insulating material onto the first.

4. A method of producing a film of insulating material on a surface comprising the steps of evaporating a first layer less than 10,000 Angstroms thick of an insulating material onto the surface, at a pressure of less than  $10^{-4}$  millimeters of mercury; raising the ambient pressure on the evaporated layer to atmospheric pressure; reducing the ambient pressure on the evaporated layer to a value less than  $10^{-4}$  millimeters of mercury; and evaporating a second layer less than 10,000 Angstroms thick of the insulating material onto the undisturbed first layer.

5. A method of producing a film of insulating material on a surface comprising the steps of evaporating a first layer of insulating material on a surface, in vacuum; admitting a dry inert gas in order to raise the ambient pressure on the evaporated layer; reducing the ambient pressure on the evaporated layer to that of a vacuum; and evaporating a second layer of the insulating material onto the first.

6. A method of producing a thin silicon monoxide film comprising the steps of:  
evaporating a silicon monoxide film onto a substrate, in vacuum;  
raising the ambient pressure on the film;  
reducing the ambient pressure on the film to that of a vacuum; and  
evaporating a second film of silicon monoxide onto the first silicon monoxide film.

7. A method of producing a silicon monoxide film on a surface comprising the steps of:  
evaporating a first film less than 5000 Angstroms thick of silicon monoxide onto the surface at a pressure of less than  $10^{-4}$  millimeters of mercury;  
admitting a dry inert gas to raise the ambient pressure

on the evaporated film to atmospheric pressure without introducing contaminants; reducing the ambient pressure on the evaporated film to a value less than  $10^{-4}$  millimeters of mercury; and evaporating a second silicon monoxide film less than 5000 Angstroms thick of insulating material onto the first silicon monoxide film.

|             |      |                     |          |
|-------------|------|---------------------|----------|
| 2,840,489   | 6/58 | Kempter et al.----- | 117—106  |
| 2,903,780   | 9/59 | Barnard -----       | 29—25.42 |
| 2,930,951   | 3/60 | Burger et al. ----- | 317—242  |
| 2,932,588   | 4/60 | Frank -----         | 117—106  |
| 5 3,025,441 | 3/62 | West -----          | 317—258  |

## FOREIGN PATENTS

580,137 8/46 Great Britain.

## References Cited by the Examiner

## UNITED STATES PATENTS

|           |      |                |           |
|-----------|------|----------------|-----------|
| 2,593,829 | 4/52 | Arledter ----- | 317—260   |
| 2,734,478 | 2/56 | Reynolds ----- | 317—258 X |

10 RICHARD D. NEVIUS, *Primary Examiner.*  
S. BERNSTEIN, JOHN P. WILDMAN, *Examiners.*